

July 18, 1939.

W. T. ALLEN ET AL

2,166,333

FLEXIBLE LEAD CONNECTION

Filed April 5, 1937



INVENTORS.  
Wallace T. Allen,  
Olav Maseng.  
Myron J. Leibold  
ATTORNEY

BY

## UNITED STATES PATENT OFFICE

2,166,333

## FLEXIBLE LEAD CONNECTION

Wallace T. Allen, Royal Oak, and Olav Maseng,  
Detroit, Mich., assignors to Square D Company,  
Detroit, Mich., a corporation of Michigan

Application April 5, 1937, Serial No. 135,013

7 Claims. (Cl. 219—12)

This invention relates to electrical instrumentalities and more particularly to flexible lead connections for electrically connecting relatively movable parts therein.

5 One object of the present invention is the provision of an improved flexible lead connection and the method of attaching the same which results in a very firm joint which may be quickly and economically made while avoiding the possibility of stiffening of the flexible conductor due to the running of the soldering material.

10 Another object of the invention is the provision of a flexible lead connection which results in a relatively firm joint between the end of the flexible conductor and the solid part while maintaining a thin wrapping about the conductor strands remote from the part to provide a binding or retaining means for them.

15 Other objects and features of the invention will be readily apparent to those skilled in the art from the following specification and appended drawing illustrating certain preferred embodiments of the invention in which:

20 Figure 1 is a vertical sectional view of an automatic electric circuit breaker employing a flexible lead according to the present invention.

25 Figure 2 is a broken off view similar to Figure 1 showing the parts in a different circuit relation.

30 Figure 3 is a view illustrating one means of providing the individual leads to be applied.

35 Figure 4 is a view showing an individual lead before attachment.

Figure 5 is a sectional view on the line V—V of Figure 4.

40 The joint and method of the present invention have been illustrated in connection with the circuit breaker disclosed and claimed in the copending applications of John G. Jackson, Serial No. 36,247 filed August 15, 1935; (now Patent No. 2,132,625, granted October 11, 1938), Serial No. 72,035 filed April 1, 1936 (now Patent No. 2,096,545, granted October 19, 1937); Serial No. 77,519 filed May 2, 1936 (now Patent No. 2,132,627, granted October 11, 1938); all entitled

45 Circuit breakers, and in the divisions and continuations of these applications. It is, of course, to be understood that the connection means and method is of general application and may be applied in any sort of electrical instrumentality where electrical connection is desired between relatively moving parts. The circuit breaker illustrated in Figures 1 and 2 comprises a metallic

50 backing portion 1 which may comprise the back wall of an outer enclosing box upon which is mounted an insulating base 2 having a metallic

5 cover 3 and an insulating cover liner and end shield 4. Generally centrally of the base is mounted a stationary contact plate 5 as by means of a stud 6 and carrying stationary contact surfaces thereon adapted to cooperate with movable 10 contact surfaces 7 upon the ends of floating conducting contact bars 8. Rectilinearly movable U-shaped members 9 are provided guided by formations on the base for movement at right angles to the back of the base and these members 10 have their longer legs provided with slots 11 receiving notches 12 in the upper edges of the bars 8. Compression springs 13 are provided intermediate the bars and the bottom of the base. Rotary handles 14 projecting through the cover 3 15 are provided mounted on shafts 15 and having interior camming surfaces including stable flat "off" portions 16 and resetting tips 17. Light handle position retaining springs 18 are provided to bias the handles into engagement with the 20 members 9.

Upon end latches at the exterior of the breaker enclosure connectors 19 are rigidly secured as by spun over portions of metallic inserts 21 which also receive terminal connectors 22. Upon the inner ends of the connectors 19 are mounted bimetallic members 23, this mounting including adjustment means indicated generally at 24. The free ends of the bimetallic members 23 serve to latch the ends of the contact bars 8 remote from 30 the contact surfaces 7 and these free ends are connected with intermediate points on the bars 8 by means of flexible leads 25 connected to the bimetallics and the bars in a manner to be hereinafter described. The chamber adjacent the 35 cooperating contacts is provided with an insulating liner 26 and with barriers 27 having slots adjacent their bottom portions closely receiving the contact bars 8.

The circuit breaker mechanism shown at the 40 top of Figure 1 is in the closed circuit or normal operating position with the circuit closed from the stationary contact plate 5 through the bar 8, flexible lead 25, bimetal 23 to the exterior of the breaker enclosure. Current may be led to the 45 contact plate 5 through what may be termed a main circuit breaker mechanism or through a solid connector, not shown. To move the mechanism shown at the top of Figure 1 to the "off" position the handle is rotated in a counter-clockwise direction by which the parts assume the position shown in reverse at the bottom of Figure 1 and in this position the flat surface 16 on the handle engages the flat surface at the 50 top of the member 9 and results in a stable man- 55

ual "off" position being attained. By this movement of the operating handle the member 9 has been cammed downwardly carrying with it the contact carrying end of the cooperating bar 8 into the position shown. In Figure 2 the automatic overload trip position of the parts is shown. Here an overload current has passed through the bimetal 23 therein shown and has flexed it upwardly releasing the latched end of the contact bar 8 whereupon the bar has rotated under the action of the compression spring 13 about its engagement with the member 9 into the position shown. In this movement the heavy compression spring 13 serves to compress the light handle biasing spring 18 and moves the handle into a position indicating the overload trip position of the circuit breaker. To reset the parts after an automatic trip the operating handle is moved as far as possible past the "off" position. As this movement proceeds the member 8 will be moved downwardly engaging the contact carrying end of the bar 8 with the bottom of the arc chamber and thereupon rotating the latching end of the bar downwardly. In its final movement when the resetting tip 17 is engaged with the top surface of the member 9 the latching end of the contact bar will be beyond the free end of the bimetal and assuming that the bimetal has in the meantime cooled sufficiently to return to its latching position, will replace the parts in manual "off" position whereupon movement of the handle to the "on" position will permit the bar 8 to move upwardly under the bias of spring 13 into engagement with its cooperating stationary contact.

In Figure 3 there is shown a continuous flexible conductor 31 about which at predetermined spaced intervals are wrapped thin strips of solder material 32. These strips are thereafter cut at a medial point as indicated at 33 which results in the formation of the individual flexible lead or conductor 34 shown in Figure 4 having strips of solder material wrapped around both its ends. It is to be noted that this method of placing the solder strip about the ends results in the formation of two wrapped ends by each wrapping and cutting operation. It is, of course, obvious that these ends may be individually applied if desired or that the double strip wrapping and cutting may be done singly at a spaced distance from the last cut end of the conductor 31.

Figure 5 illustrates a section through a wrapped end in Figure 4 and shows the interior finely stranded cable or lead 34 having a metal wrapping 32 therearound. In applying this flexible lead 34 to solid parts which, in the specific instance illustrated, are constituted by the free end of the bimetallic member 23 and an intermediate point on the contact bar 8 the wrapped end of the lead may be placed against the part at the point of attachment and the part and lead end pressed together between electrodes whereupon the passage of current through the electrodes is adjusted to fuse substantially only the portion of the wrapping placed against the fixed part leaving the outer portion intact as a wrapping about the ends of the cable strands. This fusing or brazing operation may be done with facility upon a spot welding machine.

Applicants' invention has so far been disclosed in its specific aspects. However, in its broader terms it includes the brazing of a flexible conductor end to a solid part by means of a piece of solid soldering material placed between the end of the lead and the solid part and fused by any desired method but for which the oper-

ation similar to spot welding is particularly adapted. This portion of solid solder is carefully limited in volume so that while there is produced molten solder which will flow into the strands of the cable, insufficient solder is used to permit the flowing of the solder up the strands of the conductor by capillary action such as occurs by the use of liquid soldering and which results in rendering the flexible lead stiff and more apt to break in the operation of the parts.

While applicants' invention in its broader aspect is to be construed as including the attaching of a flexible lead by the placing of a selected quantity of solid soldering material between the end of the lead and the solid part to which it is to be attached and the fusing of this portion of solder to form the bond, which selected quantity is sufficient to permit flow into the strands of the lead but insufficient to allow flow up the strands by capillary action, still the wrapping method previously described is preferred as it provides not only for the fusing of this small quantity of solder to avoid the capillary action referred to but also results in the maintaining of the wrapped strip about the portion of the lead away from the part to which it is attached which wrapping then functions as a binding to prevent strands of the cable from loosening from the joint. Applicants' invention not only avoids the necessity of any mechanically attached end, more particularly the use of a separate encasing terminal lug to which the flexible lead might otherwise have been soldered, but also avoids the flow of solder up the strands by capillary action which is hardly to be avoided in the use of a liquid solder. The construction lends itself to rapid and economical production with the attainment of a strong joint and a fully flexible lead.

While certain preferred embodiments of the invention have been specifically disclosed, it is understood that the invention is not limited thereto as many variations will be readily apparent to those skilled in the art and the invention is to be given its broadest possible interpretation within the terms of the following claims.

What is claimed is:

1. The method of attaching the end of a stranded, flexible conductor to a solid part in electrically conducting relation which comprises wrapping said conductor end with a thin strip of solid solder, applying said wrapped end to the solid part to which it is to be attached, fusing the portion of said wrapping lying against the part to firmly braze the conductor end to the part, and maintaining the portion of the wrapping away from the part in a solid state to provide a binding for the conductor strands.

2. The method of attaching the end of a stranded, flexible conductor to a solid part in electrically conducting relation which comprises wrapping said conductor end with a thin strip of solid solder, applying said wrapped end to the solid part to which it is to be attached, fusing the portion of said wrapping lying against the part to firmly braze the conductor end to the part, and maintaining the portion of the wrapping away from the part in a solid state to provide a binding for the conductor strands, the quantity of solder actually fused being insufficient to provide for flow along the conductor strands away from the point of attachment, whereby stiffening of the conductor is avoided.

3. The method of attaching the end of a stranded, flexible conductor to a solid part in

- electrically conducting relation which comprises wrapping said conductor end with a thin strip of solid solder, applying said wrapped end to the solid part to which it is to be attached, fusing the portion of said wrapping lying against the part to firmly braze the conductor end to the part, and maintaining the portion of the wrapping away from the part in a solid state to provide a binding for the conducting strands, the portion of said wrapping actually fused being sufficient to provide for solder flow into the strands at the point of attachment but insufficient to permit solder flow along the strands away from the point of attachment.
5. A unit assembly attachment between a flexible, stranded conductor and a solid part including a thin strip wrapping of solder about the end of the conductor with the portion of said wrapping immediately adjacent the part fused thereagainst and firmly brazing the conductor to the part and with the portion of said wrapping remote from the part substantially intact and providing a binding for the conductor strands.
10. 4. A unit assembly attachment between a flexible, stranded conductor and a solid part including a thin strip wrapping of solder about the end of the conductor with the portion of said wrapping immediately adjacent the part fused thereagainst and firmly brazing the conductor to the part and with the portion of said wrapping remote from the part substantially intact and providing a binding for the conductor strands, said fused portion being distributed in the conductor strands only immediately adjacent to the
15. 5. A unit assembly attachment between a flexible, stranded conductor and a solid part comprising a thin strip wrapping of solder about the end of the conductor with the portion of said wrapping immediately adjacent the part fused thereagainst and firmly brazing the conductor to the part and with the portion of said wrapping remote from the part substantially intact and providing a binding for the conductor strands.
20. 6. The method of attaching the end of a stranded, flexible conductor, composed of individual strands twisted together and of a fineness making the conductor susceptible to a substantial diffusion of molten metal along the
25. strands by capillary action from the point of application, to a substantially flat surface on a solid part in electrically conducting relation without the use of a terminal or lug which comprises selecting a portion of solid solder of a quantity to provide for flow of melted solder into the conductor strands at the point of attachment while substantially inhibiting the diffusion or flow of molten solder along the conductor strands by this capillary action, placing this solid solder between said flat surface and said conductor end, and electrically brazing said end to said part through said solder by passing current therethrough between electrodes pressed thereagainst.
30. 7. The method of attaching the end of a stranded, flexible conductor, having individual strands of a fineness making the conductor susceptible to a substantial diffusion of molten metal along the strands by capillary action from the point of application, to a substantially flat surface of a solid part in electrically conducting relation without the use of a terminal or lug which comprises placing a portion of solid solder between said conductor end and said flat surface, pressing said conductor end, solder portion and flat surface together between electrodes, and passing current between said electrodes to fuse at least a part of said solder portion, said at least a part of said solder portion being so small in volume as to inhibit the diffusion or flow of solder up the conductor strands by capillary action, thus preventing stiffening of the conductor adjacent to the joint, while providing for flow of solder into the conductor strands at the joint, thus binding them together and to said solid part.
35. WALLACE T. ALLEN.  
OLAV MASENG.